

April 18, 1939.

W. M. HINMAN ET AL

2,154,506

MANUFACTURE OF BLUE-PRINT SHEETS

Filed March 8, 1937

TOP COAT. CONTAINING LIGHT-SENSITIVE  
FERRIOXALATE SALT AND  
SOLUBLE FERRICYANIDE SALT;  
AND OPTIONAL CONTENTS OF  
REDUCING AGENT LIKE OXALATE  
SALT AND A BODY LIKE  
GELATINE.

UNDER COAT. CONTAINING SALT FROM GROUP:  
SOLUBLE FERRICYANIDE AND  
FERROCYANIDE SALTS; AND  
OPTIONAL CONTENTS OF SIMPLE  
OXALATE SALT AND BODY LIKE  
GELATINE



Inventors.  
Walker M. Hinman  
Walter G. Hollmann  
by W. Bartlett Jones,  
Attorney

## UNITED STATES PATENT OFFICE

2,154,506

## MANUFACTURE OF BLUE-PRINT SHEETS

Walker M. Hinman, Winnetka, and Walter G. Hollmann, Chicago, Ill., assignors to The Frederick Post Company, Chicago, Ill., a corporation of Illinois

Application March 8, 1937, Serial No. 129,846

15 Claims. (Cl. 95—6)

The present invention relates to blue print papers and the like of the type in which light is used to produce a blue background of complex iron cyanogen compounds from appropriate light-sensitive chemical mixtures, followed by a wetting development procedure.

The art is well known generally with many variations and the trade has attained a more or less fixed status which includes standard hand and machine operations requiring papers of specified "speed" and other characteristics. One of the difficulties heretofore encountered has been the increase in the "speed" of printing a paper without sacrifice of depth of blue color, and another aspect of the same problem, an increase in the depth of color of a given "speed" of paper. Attempts to solve these problems by increased concentrations of sensitizing solutions and increased thicknesses of sensitive coatings have reached a limited success, and then other difficulties are encountered.

The object of the present invention is to make a sensitized blue-printing sheet which has when developed an improved depth of blue at a given printing speed, or a speedier paper for a desired depth of blue.

A particular object of the invention is to use initially in the sensitive coating a product which is formed ordinarily in the light-printing operation.

Still another object of the invention is to thicken the coating by dividing it into two different but contiguous bodies or layers, and to use in one body or layer materials which need not be struck by light, while reserving for the other body or layer, materials which must be struck by light.

Various other and ancillary objects and advantages of the invention will become apparent from the following detailed explanation of the invention and of several ways of carrying it out.

The invention can best be understood by a brief reference to the fundamental chemistry of blue-print papers. Blue-print papers are dry sensitized sheets usually containing a suitable ferrioxalate salt and potassium ferricyanide. The principle of operation holds that on exposing the sensitized paper to light the ferrioxalate salt is reduced forming ferrous oxalate. This is an insoluble compound which is fixed in position in the paper and forms the pattern of the print, and is changed later in situ to an insoluble blue compound. In the presence of water the ferrous oxalate and the potassium ferricyanide react to form insoluble blue ferrous

ferricyanide. Where light does not strike the sheet the ferrioxalate remains unchanged and the original unchanged sensitizing mixture is washed out. Thus the developed sheet contains no chemical where it is protected from light, 5 and contains blue insoluble ferrous ferricyanide where it is struck by light.

However, the practical operations are not fully in accordance with this main principle, partly because there are side or additional reactions. 10 The first of these is a minor chemical reduction which takes place, principally during exposure, by action of the oxalate content of the coating on the ferricyanide, forming some theoretically undesired potassium ferrocyanide in the light-struck portion, and leaving a portion of the theoretically desirable unchanged potassium ferricyanide. Therefore on wetting the exposed print there follows another side reaction whereby the newly formed ferrous oxalate combines 20 also with the newly formed potassium ferrocyanide to form ferrous ferrocyanide, which is a white insoluble compound. It is thus seen that where theory calls for transformation of the insoluble ferrous oxalate to a blue pigment, a 25 white pigment also may be formed by the secondary reaction. Mixtures from blue to white may result. If the exposure to light is weak, the secondary reaction is less and more blue pigment forms. If the exposure to light is strong 30 the secondary reaction is greater and much more white pigment forms. In commercial practice there are mixed white and blue pigments having a greyish blue appearance at this stage. In fact, it is a practice to encourage the photochemical 35 reduction of ferricyanide salt to ferrocyanide salt by having present additional reducing agent such as an oxalate, a citrate or a tartrate, but preferably an excess of some soluble oxalate salt.

Theory at this stage calls for complete washing 40 out of soluble material, largely soluble oxalate salts, so as to leave only these mixed white and blue pigments. Then, practice calls for oxidation whereby the insoluble white ferrous ferrocyanide is converted to insoluble blue ferric ferrocyanide. Air will oxidize it, but this is too slow. Hence a chemical oxidizer is used, and such use in more perfected form is set forth in the co-pending application of applicant Hinman, Serial No. 727,248, filed May 24, 1934, the invention of 45 which is applicable to the paper made by the present invention.

Referring to the above description, it should be stated that it describes what occurs in blue-print papers having a sensitizing mixture of fer- 55

rioxalate and ferricyanide as appropriate salts. The ferrioxalate is essentially the one compound which must be decomposed or altered by light to produce ferrous oxalate. At the same time the ferricyanide is only incidentally but desirably altered, and that occurs because it is usually present with some form of reducing agent, usually the ferrioxalate or other oxalate, which furnishes the reducing power whereby a ferrocyanide is formed. But this incidental reduction utilizes some of the actinic energy which should be directed toward forming ferrous oxalate. As a result the paper is slower printing for a given depth of blue, or else the blue is weaker for a given time of printing.

According to the present invention this incidental waste of actinic energy in the light-printing period is minimized. The manner in which this is done may be presented in several aspects, 20 but generally it may be said that the essential light-sensitive ferrioxalate is more effectively concentrated near the surface of the sensitized sheet, and the ferricyanide content which ordinarily goes with it is lessened. Not only is this 25 accompanying ferricyanide content lessened by shifting its location, but the shifted portion is in whole or in part replaced by ferrocyanide and located below the top surface but contiguous thereto. And in addition, to maintain more or 30 less distinct but contiguous bodies or layers, a sizing, or matrix, or body, or vehicular substance of suitable sort may be used in one or both bodies or layers, to maintain a certain degree of isolation, at least until after the light-exposure 35 has been made.

Thus, it has been found that more of the light energy in printing may be used to form a deeper field or image of insoluble ferrous oxalate. Upon development by wetting, the chemicals of the 40 inner and outer layers readily diffuse to meet with each other. Thus the insoluble ferrous oxalate forms the blue insoluble ferrous ferricyanide, and also forms the white insoluble ferrous ferrocyanide, which latter is oxidizable in development to insoluble blue ferric ferrocyanide.

At this point it is pertinent to state that a dried paper coated only with a solution of ammonium ferrioxalate, which is the form most commonly used, is substantially colorless. The ferricyanides 50 and ferrocyanides are respectively red and yellow. By reducing in the upper body or layer the ratio of these cyanides to ferrioxalate the residual coating is less colored and less obstructive of light as a light filter, and more permeable to 55 the violet end or ultraviolet rays of the spectrum used in light printing, at which end the actinic energy is greater. These facts also add to the efficiency in use of light, and give increased "speed."

60 In the practice of the present invention it has been found that the prior art practice of having ferrioxalate and ferricyanide intimately associated, must still be observed, and the ratio of these 65 may vary greatly as in the prior art. It has not been found possible to make a complete separation as the general discussion might lead the reader up to this point to suspect. Hence, since ferricyanide must be used in the surface coat, body or layer, it is preferred to use in the lower 70 coat, body or layer ferrocyanide without ferri- cyanide, and to reduce the ferricyanide content of the surface coat, body or layer. In practice the total quantity of iron cyanides thus employed 75 in both bodies or layers may be less than has

been needed heretofore when there has been no separation into two portions.

In creating the coats, bodies or layers it becomes necessary to use something to define the same and to maintain some line of demarcation between them. This may be accomplished simply by using a gum or colloid or other coating substance which will contain the chemicals, and which when wet will permit the release or the diffusion of such chemicals from the colloid. 10 Many film-forming substances are known and may be used such as: glue, gelatine, starch, dextrine, oxidized starch, other converted or soluble starches and starch derivatives, certain cellulose derivatives, regenerated cellulose, gum arabic, 15 gum tragacanth, and a large number of gums and substances which may generally be designated as hydrophilic colloids or substances. Preferably they are used in solution form and are dried after application. Of course a paper base itself 20 may constitute a medium to define the first residue, and a second residue may be formed thereon. But usually the paper base for blue-print papers is highly sized or finished so that its surface is not at all or not very absorptive of coating 25 solutions, thus to form more nearly true coatings rather than impregnated paper surfaces. It is customary in the ordinary coating of blue-print paper to use a coating solution containing an agent of the character above specified, such as 30 glue or gelatine, partly in order to facilitate spreading of the sensitizing composition with even distribution over the sheet, and to hold it in place in developing the sheet. The present invention therefore contemplates using such 35 agent in either or in both compositions to be applied in creating bodies or layers. It is also to be considered that a body or layer may be formed in two operations as well as in one, by first applying a suitable agent such as gelatine, or even 40 regenerated cellulose, which may be dried in whole or in part, and then wetted with a solution which may contain the chemicals and may be lacking in a glue-like substance.

In practical operations under this invention a well sized paper is used. This is coated with an under-coating composition containing hydrophilic substance and certain chemicals, and then dried. The dried coating may be covered immediately or later with the surface-coating composition, and this likewise contains hydrophilic body substance by preference and the light-sensitive chemicals. If the hydrophilic body is omitted and the coating composition contains only chemicals, these enter the surface of the so-called dried under-coating to a degree, but yet contiguous superimposed coats are present, although not sharply defined. By preference therefore, an agent such as gelatine is included in each coating composition to maintain more complete separation. Also, it is preferred to dry the first coating and to coat immediately, to form the second coating, since this assures uniform surface conditions on the undercoat for receiving the second coat, whereby the dual coatings present a uniform product when continuous production is employed. Actually, one drying oven is employed for a continuous web of paper. There are two coating baths and devices, one positioned to operate on a paper web just before it enters 70 the oven, and the other positioned to operate on the dried paper web, preferably while warm or hot, and while it is temporarily taken from the drying oven. An oven temperature of 180° F. is suitable for all the solutions hereinafter dis- 75

closed, but it is to be understood that this temperature is not critical, nor is heat necessary for the process. Ordinary coating devices known to the art suffice for each coating composition.

EXAMPLE I

Under coat. Water to 100 gallons

|                                | Pounds |
|--------------------------------|--------|
| 10 Sodium ferrocyanide         | 1      |
| 10 Ammonium oxalate            | 32     |
| Potassium ferricyanide         | 6      |
| Powdered glue (adhesive grade) | 26     |

Surface coat. Water to 100 gallons

|                          | Pounds |
|--------------------------|--------|
| 15 Ammonium ferrioxalate | 175    |
| Ammonium oxalate         | 32     |
| Potassium ferricyanide   | 18     |

EXAMPLE II

Under coat. Water to 100 gallons

|                        | Pounds |
|------------------------|--------|
| Potassium ferrocyanide | 6      |
| 25 Ammonium oxalate    | 32     |
| Gelatin                | 6.5    |

Surface coat. Water to 100 gallons

|                          | Pounds |
|--------------------------|--------|
| 30 Ammonium ferrioxalate | 175    |
| Ammonium oxalate         | 8      |
| Potassium ferricyanide   | 18     |
| Gelatin                  | 0.5    |

EXAMPLE III

Under coat. Water to 100 gallons

|                               | Pounds |
|-------------------------------|--------|
| Sodium ferrocyanide           | 6.00   |
| Oxalic acid                   | 31.25  |
| 40 Ammonia (26° Bé.)          | 16.25  |
| Anhydrous potassium carbonate | 12.00  |
| Powdered glue                 | 14.25  |
| Monosodium phosphate          | 3.50   |

Surface coat. Water to 100 gallons

|                        | lbs   |
|------------------------|-------|
| Ammonium ferrioxalate  | 189   |
| Ammonia (26° Bé.)      | 7.38  |
| Monosodium phosphate   | 8.25  |
| Oxalic acid            | 7.00  |
| 50 Photoengraving glue | 630   |
| Potassium ferricyanide | 23.25 |

The above examples illustrate the wide variations possible in carrying out the invention. They include much that falls within the skill of the art. Sensitizing solutions heretofore employed include an oxalate salt, such as of sodium, ammonium, or potassium or even mixtures of such salts. They are important in retarding reactions in the coating solutions or in the coated paper until proper exposure and development, and hence maintain a more stable sensitized paper. They also provide reducing agent for the ferricyanide salt to convert it to ferrocyanide salt under the influence of light. The mono-sodium phosphate has also a retarding function, but doubtlessly through the different mechanism of hydrogen ion control by its buffer action. In Examples I and II the oxalate salts are employed as such in compounding the formula, and the ammonium salt alone is used, since it is fairly insoluble and does not so readily transfer from the dried under coat in applying the surface coating composition. In Example III these oxalate salts are built up from formative components, such as

oxalic acid, ammonia, and potassium carbonate, forming both ammonium oxalate and potassium oxalate. Slight excess of any such component is not harmful in the presence of the buffer salt monosodium phosphate, and this gives some latitude for variations of the formula by carelessness, error, or variations in material.

The accompanying drawing illustrates the invention showing particularly the arrangement of the bodies. In the drawing 10 illustrates the carrier base, which is preferably a well-sized sheet of paper as commonly used in the blueprint field, which can receive a liquid coating composition and form a residual coat when dried. Numeral 11 represents the position of the resulting dried coat, as may be readily produced from the solutions designated "Under coat" in the examples. Numeral 12 represents the position of the residue formed by coating onto the dry body 11 a composition such as that designated "Surface coat" in the examples, and drying the same. The legends on the parts indicate briefly the variations discussed hereinabove.

Returning to the pertinent phases of the invention it may be noted that some of the oxalate content of the prior art, as well as some of the iron cyanide content, has been transferred from the light-sensitive surface coat 12 to the under coat 11. Since some reducing agent in addition to the oxalate content of ferrioxalate is desirable for transforming ferricyanide to ferrocyanide, it is desirable not to move all of the oxalate or other reducing agent (citrates and tartrates being also used), into the under coat. However, the lessened concentrations of such reducing agent and of ferricyanide salt is effective to lessen the tendency for the ferricyanide to use up actinic energy in being reduced to ferrocyanide. Thus there is left a greater opportunity for the preponderating quantity of ferrioxalate to be reduced to the field-image-forming ferrous oxalate, without collateral loss caused by the presence of chemicals necessary for the later reactions of development.

From the foregoing it will be readily understood how the invention may be modified and changed from the preferred examples given. It is appreciated that different manufacturers of blue-print papers use variations of many basic formulas, and employ different combinations of various salts, usually selecting from sodium, potassium and ammonium salts. All those departures and modifications naturally occurring to those skilled in the art, and suggested herein by the nature of this disclosure, are contemplated as falling within the invention as defined by the appended claims.

We claim:

1. A sensitized blue-print sheet comprising a sheet having two contiguous water-permeable coats containing chemical ingredients, one coat being light-sensitive and located for positioning it between the other and a source of actinic light and containing light-sensitive ferrioxalate salt, a soluble ferricyanide salt and a reducing agent, therefor capable of converting the ferricyanide to ferrocyanide by the action of actinic light, and the other coat containing a soluble complex salt of the group consisting of ferricyanide and ferrocyanide which is adapted to diffuse to the first coat upon wetting for reaction with the insoluble ferrous oxalate formed in the light-sensitive coat by the action of light.
2. A sensitized blue-print sheet comprising a sheet having two contiguous water-permeable

coats containing chemical ingredients, one coat being light-sensitive and located for positioning it between the other and a source of actinic light and containing light-sensitive ferrioxalate salt, a soluble ferricyanide salt and a reducing agent therefor capable of converting the ferricyanide to ferrocyanide by the action of actinic light, and the other coat containing a soluble ferrocyanide salt which is adapted to diffuse to the first coat upon wetting for reaction with the insoluble ferrous oxalate formed in the light-sensitive coat by the action of light.

3. A sensitized blue-print sheet comprising a sheet having two contiguous water-permeable coats containing chemical ingredients, one coat being light-sensitive and located for positioning it between the other and a source of actinic light and containing light-sensitive ferrioxalate salt, a soluble ferricyanide salt and a reducing agent therefor capable of converting the ferricyanide to ferrocyanide by the action of actinic light, and the other coat containing a soluble ferrocyanide salt and a soluble ferricyanide salt both of which are adapted to diffuse to the first coat upon wetting for reaction with the insoluble ferrous oxalate formed in the light-sensitive coat by the action of light.

4. A sensitized blue-print sheet comprising a sheet having two contiguous water-permeable coats containing chemical ingredients, one coat being light-sensitive and located for positioning it between the other and a source of actinic light and containing light-sensitive ferrioxalate salt, a soluble ferricyanide salt and a reducing agent therefor capable of converting the ferricyanide to ferrocyanide by the action of actinic light, and the other coat containing a soluble oxalate salt, and also a soluble ferrocyanide salt and a soluble ferricyanide salt both of which are adapted to diffuse to the first coat upon wetting for reaction with the insoluble ferrous oxalate formed in the light-sensitive coat by the action of light.

5. A sensitized blue-print sheet comprising a sheet having two contiguous water-permeable coats containing chemical ingredients, one coat being light-sensitive and located for positioning it between the other and a source of actinic light and containing light-sensitive ferrioxalate salt and a soluble ferricyanide salt as the essential ingredients for reaction under the influence of actinic light to produce insoluble ferrous oxalate, and the other coat containing a supply of soluble salt of the group consisting of ferricyanide and ferrocyanide essential for the development of an insoluble pigment upon application of water, by diffusion to and reaction with the ferrous oxalate.

6. A sensitized blue-print sheet containing a sheet having two contiguous water-permeable coats containing chemical ingredients, one coat being light-sensitive and located for positioning it between the other and a source of actinic light and containing light-sensitive ferrioxalate salt, and a soluble ferricyanide salt as the essential ingredients for reaction under the influence of actinic light to produce insoluble ferrous oxalate, and the other coat containing a supply of soluble salt of the group consisting of ferricyanide and ferrocyanide essential for the development of an insoluble pigment upon application of water, by diffusion to and reaction with the ferrous oxalate, each of said coats being more or less definite and containing a body of hydrophilic substance housing the respective chemical ingredients.

7. A light-sensitive sheet for blue-printing comprising a light-sensitive material in extended

sheet-like form adapted to be exposed to a source of light and containing essentially a light-sensitive mixture of soluble salts of ferrioxalate and ferricyanide, and contiguous material in like form positioned in the sheet to be more remote from said source of actinic light than said first form, said second form containing a soluble ferrocyanide salt, both materials being permeable to water to cause diffusion of ferrocyanide from the second form to the first form for development of a light-exposed print.

8. A sensitized blue-print body comprising a carrier base having two contiguous water-permeable layers thereon containing chemical ingredients, one layer being light-sensitive and located for positioning it between the other and a source of actinic light and containing light-sensitive ferrioxalate salt, a soluble ferricyanide salt and a reducing agent therefor capable of converting the ferricyanide to ferrocyanide by the action of actinic light, and the other layer containing a soluble complex salt of the group consisting of ferricyanide and ferrocyanide which is adapted to diffuse to the first layer upon wetting for reaction with the insoluble ferrous oxalate formed in the light-sensitive layer by the action of light.

9. A sensitized blue-print body comprising a carrier base having two contiguous water-permeable layers thereon containing chemical ingredients, one layer being light-sensitive and located for positioning it between the other and a source of actinic light and containing light-sensitive ferrioxalate salt, a soluble ferricyanide salt and a reducing agent therefor capable of converting the ferricyanide to ferrocyanide by the action of actinic light, and the other layer containing a soluble ferrocyanide salt and a soluble ferricyanide salt both of which are adapted to diffuse to the first layer upon wetting for reaction with the insoluble ferrous oxalate formed in the light-sensitive layer by the action of light.

10. A sensitized blue-print body comprising a carrier base having two contiguous water-permeable layers thereon containing chemical ingredients, one layer being light-sensitive and located for positioning it between the other and a source of actinic light and containing light-sensitive ferrioxalate salt, and a soluble ferricyanide salt as the essential ingredients for reaction under the influence of actinic light to produce insoluble ferrous oxalate, and the other layer containing a supply of soluble salt of the group consisting of ferricyanide and ferrocyanide essential for the development of an insoluble pigment upon application of water, by diffusion to and reaction with the ferrous oxalate, each of said layers being more or less definite and containing a body of hydrophilic substance housing the respective chemical ingredients.

11. The process of making sensitized bodies for blue-prints of the type in which a light-sensitive ferrioxalate salt is altered by light to produce insoluble ferrous oxalate and in which a soluble complex salt of the group consisting of ferricyanide and ferrocyanide unites with the ferrous oxalate to form an insoluble complex iron iron-cyanide when water is applied, the steps of coating a carrier body with an aqueous coating composition containing salt from said above-mentioned group, drying the application to a coat on said body, then applying to said coat a second aqueous coating composition carrying a light-sensitizing substance including essentially light-sensitive ferrioxalate salt, a lesser quantity of soluble ferricyanide salt, and a reducing agent

which is capable of converting the last-mentioned ferricyanide salt to a ferrocyanide salt by the action of actinic light, and drying said second application to a coat overlying the first coat, while preserving the light-sensitive character of the resulting overlying coat.

12. The process of claim 11 in which the first coating composition includes a simple oxalate salt.

10 13. The process of claim 11 in which at least one of the coating compositions contains a film-forming hydrophilic substance as a body defining the resulting coat.

15 14. The process of making sensitized bodies for blue-prints of the type in which a light-sensitive ferrioxalate salt is altered by light to produce insoluble ferrous oxalate and in which a soluble complex salt of the group consisting of ferricyanide and ferrocyanide unites with the ferrous

oxalate to form an insoluble complex iron iron-cyanide when water is applied, the steps of coating a carrier body with an aqueous coating composition containing salt from said above-mentioned group, drying the application to a coat on said body, then applying to said coat a second aqueous coating composition carrying a light-sensitizing substance including essentially light-sensitive ferrioxalate salt and a lesser quantity of soluble ferricyanide salt, and drying said second application to a coat overlying the first coat, while preserving the light-sensitive character of the resulting overlying coat.

15 15. The process of claim 14 in which at least one of the coating compositions contains a film-forming hydrophilic substance as a body defining the resulting coat.

WALKER M. HINMAN.

WALTER G. HOLLMANN.